

1

2,941,466

## PLANOGRAPHIC PRINTING PLATES

Douglas A. Newman, Glen Cove, and Allan T. Schlotzauer, Locust Valley, N.Y., assignors to Columbia Ribbon & Carbon Manufacturing Company, Inc., Glen Cove, N.Y., a corporation of New York

No Drawing. Filed Aug. 24, 1956, Ser. No. 605,963

3 Claims. (Cl. 101—149.2)

This invention relates to planographic printing and especially to planographic printing plates formed by a coating on a flexible fibrous foundation such as paper.

In the preparation of plates of this character it has been found that coating compositions including as a film-forming ingredient a hydrophilic binder of the class of carboxymethyl cellulose compounds or compounds of other polysaccharide carboxy ethers, have the hydrophilic-oleophilic balance to give particularly good printing results. Such coatings are rendered effective as printing surfaces when the film former is insolubilized, either by a reagent included in the coating mixture, or after-applied to the dried coating. The use of certain appropriate reagents for insolubilization, particularly copper, iron, aluminum and chromium compounds, and especially chromium compounds, result in production of outstandingly good printing surfaces when reacted with the film former and aged for short periods, giving under such conditions exceptionally large numbers of good quality copies from the plate. Plates thus prepared and constituted, however, have after prolonged storage sometimes demonstrated a tendency to become overly sensitive so that they pick up ink in the background areas during printing. Apparently this is especially the case when the plates have been stored under conditions of heat together with humidity. As a result the printing quality of plates of the type in question, while uniformly high at the time of manufacture, is not predictable at a later date.

It is an object of the present invention, therefore, to provide coated flexible planographic printing plates of the type heretofore described, but improved in such a way that the tendency to become sensitive to the ink under certain storage conditions is markedly reduced or altogether eliminated.

According to commercial practice, the coatings employed on coated paper planographic printing plates usually include one or more of various fillers to improve their printing and especially their image-retentive properties. The fillers sometimes used for this purpose are china clay, barium sulphate, hydrated alumina, calcium carbonate, zinc oxide, titanium dioxide, fluorspar, fuller's earth and other similar materials.

According to the present invention, it has been discovered that, in coatings of polysaccharide carboxy ether compounds insolubilized with the salts and compounds heretofore mentioned, the presence in particular of an oxide of zinc, titanium, magnesium or calcium, or mixtures of these particular oxides, in the composition in contrast to the other materials currently used as fillers, in some manner not altogether understood at present, has a pronounced inhibiting effect on the tendency of the coatings to become sensitive with age. It is found that, regardless of storage conditions of heat and humidity, the plates which include, as a significant portion of the filler, one or more of the oxides named will be uniformly usable and capable of producing copies of acceptable grade after a period of aging.

The present invention, therefore, is characterized by the presence of an aging sensitization inhibitor in the form

2

of material selected from the group consisting of the oxides of zinc, titanium, magnesium and calcium and mixtures thereof, as a significant portion of the filler in coatings of the polysaccharide carboxy ether type, insolubilized by salts or compounds of copper, aluminum, iron and chromium, and especially compounds of chromium.

Other features and advantages will hereinafter appear.

In practicing the present invention, a flexible paper foundation sheet is preferably treated in a known manner with wet strength-imparting ingredients such as melamine formaldehyde, although this may be dispensed with in the preparation of plates for certain short-run purposes. Likewise, known surface sizings or water-barrier coatings may be applied which provide for improved operation under long-run conditions. When such preliminary preparations, if any, are completed, the paper is coated on at least one surface with one or more coats of a planographic surfacing composition.

For this purpose an aqueous suspension or slurry is prepared containing between one and five percent of a film-forming constituent such as carboxymethyl cellulose, or other polysaccharide carboxy ether, such as the carboxy ethers of starch, or carboxy ethers of the water-soluble gums containing saccharid units, such as gum arabic, gum tragacanth, mesquite gum, larch gum, etc. In addition, the suspension includes a filler which may be about two to four times the weight of the binder present. Heretofore this filler has often consisted entirely of china clay or the like, but according to the present invention, at least a certain percent of the filler is composed of an aging sensitization inhibitor in the form of an oxide of zinc, titanium, magnesium or calcium, or a mixture of two or more of these materials. Other ingredients may be included to aid, for example, in the coating operation, or for other special purposes, but the ingredients enumerated are the essentials. The slurry is applied to the paper, for example by a brush coating operation, and allowed to dry.

One example of a coating suspension for this purpose is:

### Formula I

| Ingredients:                                            | Parts by weight |
|---------------------------------------------------------|-----------------|
| 5% aqueous dispersion of sodium carboxymethyl cellulose | 100             |
| China clay                                              | 15              |
| Zinc oxide                                              | 5               |
| Glycerine                                               | 3               |

When the coating is substantially dry, the coated surface of the sheet is treated, as by tub sizing, with an aqueous solution of one or more of the metal salts or compounds heretofore mentioned. For best results a mixture of chlorides or sulfates of aluminum, ferric iron and copper, together with chromium trioxide, are employed as disclosed in the patent to Douglas A. Newman, No. 2,655,864. The preferred formula as shown in said patent is as follows:

### Formula II

| Percent           |
|-------------------|
| Copper sulphate   |
| Aluminum sulphate |
| Ferric chloride   |
| Chromium trioxide |

This treatment renders the coating insoluble in water, and the dried coating will then accept and retain imaging material and print copies of high quality when used as the plate or master in a planographic printing process.

While the two step treatment of the printing surface is very effective, there has also been discovered a means whereby substantially equivalent printing quality can be achieved using a single coating formula which automatically becomes insoluble on drying, and the present in-

vention is equally applicable to coatings of this type. An example of a coating composition according to this form of the invention is as follows:

## Formula III

|                                 |       |     |
|---------------------------------|-------|-----|
| Sodium carboxymethyl cellulose  | grams | 2.5 |
| Water                           | cc    | 78  |
| Methanol                        | cc    | 12  |
| Clay                            | grams | 7.5 |
| Zinc oxide                      | do    | 2.5 |
| Glycerine                       | do    | 1.0 |
| 5% ammoniacal copper sulphate   | cc    | 40  |
| Ammonium dichromate, C.P.       | grams | 1.0 |
| Ferric ammonium citrate, U.S.P. | do    | 1.5 |

The slurry of Formula III is applied to the paper web, as by brush coating, and allowed to dry, preferably with the application of heat, to give a coating which is water insoluble and provides a planographic printing surface of good quality.

It can be seen that both the form of the invention exemplified by Formulas I and II and that exemplified by Formula III relate to polysaccharide carboxy ether coatings which are rendered insoluble by a particular group of metal salts or compounds, and including especially, although not necessarily, a compound of chromium. The plates thus constituted may be aged for extended periods, even under adverse conditions of high temperature and humidity, and may then be successfully imaged and used to print copies of good quality. The tendency heretofore experienced for the reaction product of insolubilization treating materials such as copper, aluminum or iron salts or chromium compounds with film formers of the polysaccharide carboxy ether type to become increasingly ink sensitive with prolonged aging, presumably due to sustained subjection to heat and humidity, is found to be effectively inhibited by the presence of the special oxide filler which acts to maintain the originally manufactured and normally aged condition of the plate surface, free from unusual ink sensitivity, regardless of the duration and temperature-humidity conditions of storage which the plate may encounter.

Formula I and Formula III have been presented showing the desensitization inhibitor as zinc oxide and represent the form of the invention at present preferred from the standpoint of cost and availability. It will be understood, however, that formulas which differ from these essentially by a substitution of a substantially equal amount of titanium dioxide, magnesium oxide or calcium oxide, or of such of the more complex oxide compounds of these metals, e.g. peroxides or sesquioxides, as are commercially available, or any mixture thereof, are equally good examples of the invention and will provide compositions demonstrating in full the stated advantages.

The proportion of the special oxide filler which should be included may vary, but it has been found that the use of amounts equivalent to about thirty percent of the weight of the film former present will produce clearly noticeable effects for the purpose. In most cases it appears that no particular advantage accrues from including amounts in excess of the weight of film forming material although more may be used if desired without substantial detriment.

While the invention herein has been described with particular reference to incorporation of the special oxide filler directly in the polysaccharide carboxy ether coating mix, it has also been found that if the same is included instead in a coating which directly underlies the polysaccharide carboxy ether coating, the sensitization inhibiting advantages heretofore set out will be attained to a substantially equal extent. When the special oxide filler is thus incorporated, it appears that somewhat less than all of the special oxide material used is effective. Accordingly the amount to be employed may be calculated on the basis of what amount would give the de-

sired results if placed directly in the surface coating planned, and then preferably using a somewhat increased amount in the undercoating. For this purpose, an increase of between fifty percent and one hundred percent above the amount of special oxide filler which would have been used in the surface coating is at present recommended. It will be appreciated also that a portion of the special oxide filler may be included in both coatings if desired with equivalent beneficial effect. In fact, the inclusion of the special oxide filter in any part of a printing surface layer consisting of the printing surface coating and the coating, if any, directly underlying it will give a result demonstrating the beneficial effect heretofore noted.

Variations and modifications may be made within the scope of the claims and portions of the improvements may be used without others.

We claim:

1. A planographic printing plate comprising a fibrous flexible foundation web; a printing surface coating on said web consisting essentially of an insoluble hydrophilic polysaccharide carboxy ether film forming material insolubilized by reaction with a metal compound selected from the group consisting of copper salts, iron salts, aluminum salts and chromium compounds and which thus reacted has a hydrophilic-oleophilic balance suitable for direct-imaging use, and which is subject to becoming excessively ink-sensitive upon subsequent exposure to protracted conditions of abnormal heat and humidity, said coating including an amount of zinc oxide sufficient to act as an aging sensitization inhibitor for said insolubilized film former, said amount being equivalent to at least about thirty percent of the weight of said film forming material.

2. A planographic printing plate comprising a fibrous flexible foundation web; a printing surface coating on said web consisting essentially of an insoluble hydrophilic polysaccharide carboxy ether film forming material insolubilized by reaction with metal compounds consisting of copper, iron and aluminum salts, and a chromium compound and which thus reacted has a hydrophilic-oleophilic balance suitable for direct-imaging use, and which is subject to becoming excessively ink-sensitive upon subsequent exposure to protracted conditions of abnormal heat and humidity, said coating including a quantity of inert filler and a sufficient amount of zinc oxide to act as an aging sensitization inhibitor for said insolubilized film former, said amount being equivalent to at least about thirty percent of the weight of said film forming material.

3. A planographic printing plate comprising a fibrous flexible foundation web; a printing surface coating on said web consisting essentially of an insoluble hydrophilic polysaccharide carboxy ether film forming material insolubilized by reaction with metal compounds consisting of copper, iron and aluminum salts, and a chromium oxide compound and which when thus reacted has a hydrophilic-oleophilic balance suitable for direct-imaging use, and which is subject to becoming excessively ink-sensitive upon subsequent exposure to protracted conditions of abnormal heat and humidity, said coating including a filler which is an aging sensitization inhibitor, said inhibitor being zinc oxide present in an amount equal to at least about thirty percent of the weight of said film forming material.

## References Cited in the file of this patent

## UNITED STATES PATENTS

|    |           |                 |               |
|----|-----------|-----------------|---------------|
| 70 | 2,542,784 | Van Dusen       | Feb. 20, 1951 |
|    | 2,598,189 | Mullen          | May 27, 1952  |
|    | 2,635,537 | Worthen         | Apr. 27, 1953 |
|    | 2,655,864 | Newman          | Oct. 20, 1953 |
|    | 2,693,145 | Mullen          | Nov. 2, 1954  |
| 75 | 2,778,301 | Brimnick et al. | Jan. 22, 1957 |